

# UNITED STATES PATENT OFFICE.

JAMES GAYLEY, OF BRADDOCK, PENNSYLVANIA.

## BLAST-FURNACE LINING.

SPECIFICATION forming part of Letters Patent No. 463,146, dated November 17, 1891.

Application filed July 28, 1890. Serial No. 360,227. (No specimens.)

*To all whom it may concern:*

Be it known that I, JAMES GAYLEY, of Brad-  
dock, in the county of Allegheny and State of  
Pennsylvania, have invented a new and use-  
ful Improvement in Blast-Furnace Linings, of  
which the following is a full, clear, and exact  
description.

In constructing a blast-furnace the inclos-  
ing walls have heretofore been made of a re-  
fractory quality of fire-brick. In the lower  
portion, commonly known as the "hearth" and  
"bosh," it is of great importance that the  
brick-work should be maintained as nearly as  
possible to its original thickness, for as the  
wear increases there is increased irregularity  
in the conduct of the process which entails  
greater expense; but in this portion the wear  
is very rapid by reason of the chemical action  
of the molten cinder, which, under the intense  
heat, has a corrosive and destructive action  
on the brick-work. The wear at the bosh I  
have found to be especially injurious to the  
action of the furnace. As the brick-work be-  
comes corroded there is substituted, however,  
through the nature of the reactions of the  
blast-furnace process, a more refractory ma-  
terial, composed largely of carbon, which to  
some extent arrests this destructive action.  
It is to this carbon coating that the endurance  
of the hearth and bosh walls is due. I have  
repaired walls that were originally thirty-six  
inches thick where but six inches of the  
original brick-work remained, which were  
protected by such carbon coating of a thick-  
ness of eighteen inches. When the furnace-  
lining is new and before the carbon coating  
can have had time to form, the deterioration  
of the walls at the bosh and hearth is very  
rapid, and during the work of the furnace the  
character of the charge is apt to vary at times  
and to produce a corrosive cinder of such  
chemical nature as will eat away the natural  
carbon coating and will attack the brick walls.  
It has occurred to me that the furnace-walls  
would be much better preserved if the natural  
process of carbon deposit could be assisted  
and supplemented by constructing the walls  
of the hearth and bosh (and preferably also  
the bottom of the hearth) of a strong and du-  
rable material containing carbon in suitable  
form. The difficulty of accomplishing this is  
to secure graphitic material sufficiently strong

to resist the weight of the furnace-walls and  
the scoring action of the stock as it descends  
in the furnace. These difficulties I have over-  
come by my invention, which consists in con-  
structing the walls of the bosh and hearth of  
brick compounded of refractory fire-clay and  
graphitic carbon, such as the substances  
known in commerce as "plumbago," "black  
lead," and "graphite." The fire-clay forms a  
bond for the carbon, giving the bricks the nec-  
essary strength and durability to resist com-  
pression and abrasion, while making it in the  
form of bricks or blocks enables it to be built  
in a strong and substantial manner in the  
furnace-walls.

To make the bricks I prefer to proceed as  
follows: In an ordinary pug-mill or dry-pan I  
mix fire-clay and the graphitic carbon above  
mentioned in proportions which may be from  
twenty-five to fifty per centum of graphitic car-  
bon and from fifty to seventy-five per centum  
of fire-clay. The most desirable proportions  
I have found to be about twenty-five per  
centum of graphitic carbon and seventy-five  
per centum of fire-clay, though my invention  
is not limited to any special proportions of the  
parts, which may be varied according to the  
judgment of the skilled furnace engineer. 75  
This compound I temper and mold into the  
form of bricks suitable for building in fur-  
nace-walls and burn them in the usual manner  
in the manufacture of fire-brick, and in this  
operation it will be found that no sensible 80  
deterioration is caused by combustion of the  
carbon. I then build these bricks in the in-  
walls of the hearth and bosh of the furnace  
and in the bottom of the hearth, for example,  
so that they shall constitute eighteen inches, 90  
more or less, of the thickness of the walls, and  
in setting them I may use as a mortar a mix-  
ture of fire-clay and carbon compounded sub-  
stantially in the manner and in proportions  
as above stated. The strength of the bricks is 95  
such that they do not weaken the structure  
of the furnace, and in their practical use I  
have found them of great benefit in preserv-  
ing the walls, and consequently in making the  
work of the furnace uniform and economical. 100  
When the furnace is first started into blast,  
instead of presenting bare hearth and bosh  
walls liable to be corroded by the cinder, the  
carbon bricks resist this action of the cinder

and are themselves renewed and supplemented by the natural deposit of carbon in the furnace. The saving which I thus secure is very considerable and will be appreciated by those who practice my invention.

In making brick for the boshes I may substitute for the graphitic carbon other forms of carbon—such as pulverized anthracite coal, charcoal, or coke—though bricks thus made are not so strong or durable.

As an additional improvement I may add to the compound of which the bricks are made some lime or other basic material, such as magnesia, which may amount to about twenty 15 per centum or less of the whole mass if lime be used and five per centum or less if magnesia is used. This will render the bricks still more refractory and durable; but my invention, broadly considered, covers the bricks, 20 whether containing the basic material or not.

I claim—

1. A blast-furnace having in the in-walls of its bosh bricks containing refractory clay and carbon, substantially as and for the purposes described.

2. A blast-furnace having in the in-walls of its bosh and hearth bricks containing refractory clay and graphitic carbon, substantially as and for the purposes described.

3. A blast-furnace having in the in-walls of its bosh and hearth bricks containing refractory clay and carbon set in mortar of similar composition, substantially as and for the purposes described.

In testimony whereof I have hereunto set 35 my hand this 24th day of July, A D. 1890.

JAMES GAYLEY.

Witnesses:

W. B. CORWIN,

THOMAS W. BAKEWELL.